

## UNITED STATES PATENT OFFICE

2,117,289

## METHOD OF PREPARING A SURFACE

David A. Bosley, Jr., Lakewood, Ohio, assignor to  
The Glidden Company, Cleveland, Ohio, a cor-  
poration of Ohio

No Drawing. Original application May 26, 1933,  
Serial No. 673,107. Divided and this applica-  
tion December 17, 1934, Serial No. 757,892

3 Claims. (Cl. 91—68)

This application is a division of applicant's co-  
pending application Serial #673,107, filed May 26,  
1933.

This invention relates to priming paints for  
use over metal and other surfaces, and has par-  
ticular reference to an improved method of for-  
mulating such products for use under sanding  
surfaces, and more particularly to a method of  
finishing surfaces by the use of my new priming  
paints. It contemplates a radical departure from  
old pigment combinations used in these materials.

When high-grade finishes are to be applied to  
surfaces, it is common practice to include three  
types of coatings in the finishing schedule: a  
primer, for adhesion and rust inhibition; one or  
more surfacing coats, to be surfaced by a sanding  
or similar operation; and one or more finishing  
coats, as a protective and ornamental finish.  
The finishing coats are very often sanded and  
polished; this is particularly true in the nitro-  
cellulose lacquer enamel finishing of automobiles  
and similar objects. The repeated sanding opera-  
tions very often abrade the surface to the  
primer; and with the primers in common use  
heretofore, the surface is often cut down clear  
to the metal. This necessitates the spotting in  
of a touch-up primer, and the building up of the  
system anew—an expensive, time-wasting series  
of operations. Furthermore, while most primers  
are baked, the touch-up primer is generally of an  
air-drying nature, and is a source of potential  
trouble in service.

My invention consists, basically, in formulating  
the primer so that, on sanding of the top coats,  
when the primer is reached, it will resist the  
action of the abrasive, and tend to abrade the  
sand-paper or sanding wheel to the same extent  
as the sand-paper abrades the primer, or to a  
greater degree. I accomplish this by incorpo-  
rating into the primer a pigment as hard as, or  
harder than, the abrasive to be employed. Since  
a primer vehicle generally holds its pigment much  
more tightly than the abrasive is held to the  
paper, and the abrasive cannot scratch the pig-  
ment, it is either abraded itself, or dusted off  
from the paper or wheel, falling or being me-  
chanically swept off the surface by the operator.

In the formulation of primers of the prior art,  
various vehicles have been used, including nitro-  
cellulose lacquers, varnishes of natural and syn-  
thetic gums, and synthetic resin solutions. Pig-  
ments of three classes have been employed with  
these vehicles; rust inhibitive pigments, such as  
red lead and zinc chromate, etc.; covering pig-  
ments, such as lithopone, zinc oxide, white lead,  
iron oxide, etc.; and cheap non-covering inert  
pigments which give filling. These pigments  
have been dispersed in the vehicles in various  
types of paint grinding equipment, including  
buhrstone, pebble and steel roll mills. In order  
to get easy dispersion, and to minimize abrasive  
action of the mills, the paint industry has always  
preferred soft pigments. The covering and rust-  
inhibitive pigments are generally manufactured  
and are very soft; a hardness of above 2.5 on the  
Moh scale is very rare. The milled pigments,  
iron oxide, the umbers and siennas, etc. are some-  
what harder; but the softer grades are preferred  
for paint work, and it may be concluded that  
these pigments do not exceed 5 in hardness. The  
softer inert—magnesium silicate, kaolin and barytes  
do not exceed 2.5—calcite has a hardness of 3 and the various talcs may be as  
low as 1 in hardness. The only common inert  
of any appreciable hardness is silica, which is #7  
on Moh's scale. This has been used in primers  
heretofore in small quantities; because of its  
tendency to abrade the mill linings, a fine grind  
was never attempted, and the slightly coarser  
silica particles were used to give the primer tooth,  
i. e. a slightly roughened surface so that the next  
coat would have good adhesion to the primer.  
Larger quantities were not employed, because of  
the heightened action on the mill linings, and  
the apparent lack of utility.

Sand-paper and sanding wheels, used for sur-  
facing, were formerly prepared with silica sand  
(hardness 7); but the newer wheels employ sili-  
con carbide (carborundum) and aluminum oxide  
(alundum) which have hardness of approxi-  
mately 9. When these abrasives come into contact  
with primers containing the soft pigments com-  
monly used, a very rapid sanding action is ob-  
tained, with resultant necessity for touch-up  
work.

By adding to a primer larger quantities of silica,  
2 to 4 pounds per gallon, a primed surface is  
obtainable which is not abraded by the silica type  
papers, and resists to a considerable degree the  
silicon carbide and aluminum oxide types. The  
use of smaller quantities of aluminum oxide and  
silicon carbide powders (1/2 pound to 1 1/2 pounds)  
gives primers which are superior to the silica type  
primer for use with the harder abrasives, and  
equal for use with the silica abrasive.

In formulation of primers with these hard pig-  
ments, the general principles of primer formula-  
tion should be employed. The vehicle should have

good adhesion, and resist lifting by the top coats, without being too hard to prevent adhesion; any of the present vehicles may be employed successfully, except the very soft or very short types.

5 There is a tendency, when the two abrasives in primer and paper meet for the engagement to cause a strain on the vehicle and on the adhesive; if the vehicle is too soft, the abrasive in the primer may tear through the vehicle; if the 10 vehicle is too short, the bond of the abrasive may be better than the bond of the primer.

The common rust-inhibitive and covering pigments may be employed as in ordinary formulation; the hard pigments are inerts, and should 15 replace the softer inerts to a greater or lesser degree. Wherever silica is hard enough, it may be used as the only hard inert; for general use, however, it is preferable to add a harder pigment to resist the action of the harder abrasives.

20 The use of these harder materials presents a very serious maintenance problem. Even where smaller quantities of silica were used to give tooth, the amount was held at a minimum to reduce the wear on mill facings. To overcome this 25 difficulty which would be very serious with the amounts I use, I prepare my primer with any desired combination of pigment and vehicle, in any type of mill. To the thoroughly ground primer, which has been transferred to a mixer, I add 30 the hard pigment in the form of a very fine dust, using as fine a material as is economically obtainable. The resultant primer is then carefully mixed; and a satisfactory degree of dispersion for primer work can be obtained by this method.

35 The following examples are typical of my invention:

*I. Light brown primer—overnight air dry*

|                                            |        |       |
|--------------------------------------------|--------|-------|
| Blown linseed oil                          | pints  | 1     |
| 40 10 gal. East India gum-wood oil varnish | do     | 3 1/2 |
| Solvent naphtha                            | do     | 1     |
| Petroleum naphtha                          | do     | 2 1/2 |
| Black magnetic iron oxide                  | pounds | 3/4   |
| Chrome orange                              | do     | 3 1/2 |
| 45 Magnesium silicate                      | do     | 2     |

Grind together on stone mill to good B grind, add silica (300 mesh—3#). Run through mill once. The silica in this case is not fine enough to wet thoroughly by merely mixing. The primer has 50 fair resistance to abrasive action.

*II. Oxide baking primer*

|                                      |        |       |
|--------------------------------------|--------|-------|
| 25 gallon wood oil ester gum varnish | pints  | 5     |
| 55 Heat bodied perilla oil           | do     | 1     |
| VM & P naphtha                       | do     | 1     |
| Turpentine substitute naphtha        | do     | 1     |
| Guaiacol (anti-oxidant)              | ounce  | 1/4   |
| Persian gulf oxide                   | pounds | 1 1/4 |
| 60 Lamp black                        | ounces | 5     |
| Soft siliceous inert                 | pound  | 3/4   |

This is given an A grind in a pebble mill. After grinding, 1 gallon of varnish is mixed with every 55 gallons of primer, and to each gallon of the

mixture is added 1/4 pound of 600 mesh silicon carbide flour, which wets satisfactorily by merely mixing. This primer is very resistant to the action of sand-paper and sanding wheels; when used as a baking oxide primer under surfacer on 5 automobile bodies it reduces cutting through to the metal to a negligible factor.

III.—A primer made exactly like the last, except substituting aluminum oxide powder for the silicon carbide powder, also gives satisfactory re- 10

While the examples given show only ordinary varnish and oil vehicles, it is possible to formulate these primers with vehicles containing phenol-aldehyde and alkyd type resins, and get excellent results, always bearing in mind that the vehicle should not be soft, or very short.

Better results are obtained in formulation of primers according to my invention, if the total quantity of pigment is kept reasonably low (3-4 20 pounds per gallon of vehicle); this permits of better anchorage in the vehicle for the hard pigment particles to resist the action of the abrasives.

I know of no common, cheap materials for use 25 as hard pigments in primer other than the products mentioned. The very hard gems (topaz, beryl, diamond, tourmaline, zircon and spinel) with a hardness of 7.5 or higher, could of course be employed with results varying with the hardness; 30 but they are all too expensive for consideration. Any pigment as hard as or harder than the abrasives commonly employed in sanding, would come within the scope of my invention.

The novel priming compositions disclosed here 35 are claimed in my co-pending application Serial #673,107, filed May 26, 1933. I claim herein only the method of preparing the surface, using my novel priming compositions in conjunction with the proper type of abrasive.

Having described my invention, I claim:

1. The method of preparing a surface which consists in applying a primer containing as an essential ingredient silicon carbide, applying over the primer a sanding surfacer, drying the surfacer, and smoothing the surface with an abrasive which will abrade the surfacer without substantially affecting the primer.

2. The method of preparing a surface which consists in applying a primer, containing as an 50 essential ingredient aluminum oxide (alundum), applying over the primer a sanding surfacer, drying the surfacer, and smoothing the surface with an abrasive which will abrade the surfacer without substantially affecting the primer.

3. The method of preparing a surface which consists in applying a primer containing as an essential ingredient a pigment as hard as or harder than silicon carbide (carborundum) and aluminum oxide (alundum), applying over the 60 primer a sanding surfacer, drying the surfacer, and smoothing the surface with an abrasive which will abrade the surfacer without substantially affecting the primer.

DAVID A. BOSLEY, JR. 65